# EUROPEAN PATENT SPECIFICATION

(11) **EP 3 258 011 B1**
(45) Date of publication and mention of the grant of the patent: **03.03.2021**
(21) Application number: 17176510.0
(22) Date of filing: 16.06.2017
(51) Int. Cl.: E01B 31/18

(54) **IN SITU REPAIRING OF A DEFECT IN A RAILWAY RAIL**
VERFAHREN ZUM REPARIEREN VON SCHIENEN EINES GLEISES VOR ORT
PROCÉDÉ DE RÉPARATION SUR PLACE DE RAILS DE CHEMIN DE FER

(30) Priority: 16.06.2016 NL 2016983
(43) Date of publication of application: 20.12.2017
(73) Proprietor: VolkerWessels Intellectuele Eigendom B.V., 3826 PA Amersfoort (NL)
(72) Inventor: Arts, Thomas, 4131 NJ Vianen (NL); van Buuren, Henrie, 4131 NJ Vianen (NL)
(74) Representative: Nederlandsch Octrooibureau

(56) References cited:
- WO-A1-2011/119238
- WO-A2-2004/014708
- FR-A- 772 282
- US-A- 619 013

## Description

This invention relates to a method of in situ repairing a mechanical defect in a rail of an existing train track for transporting passengers or goods with two parallel steel rails for rail traffic. The invention also relates to a rail obtained by a method of in situ repairing a mechanical defect in an existing rail.

Optionally, the invention is applicable to crane track rail.

From WO2011119238A1, it is known to remove a wedge-shaped piece from the rail situated in the railroad, in such a way that the rail foot and the lower part of the rail web and along a length of the rail head and the upper part of the rail web remain unaffected and for some length the rail head and the upper part of the rail web are removed completely, to then be filled by an identical prefabricated, dimensionally stable (or shape-stable), and wedge-shaped plug of steel that is permanently welded to the surrounding rail to restore the original geometry of the rail. The steel type and hardness of the plug and the rail to be repaired are the same.

US-A-619 013 (published 1899) discloses the preventive, in the vicinity of an expansion joint in the rail, and at a fixed distance therefrom in the longitudinal direction of the rail, in the tread band of the rail head positioning of a prefabricated, cylindrical, smooth-walled plug of metal harder than the rail itself, in order to absorb impact of the train wheels in the vicinity of expansion joints in the rail. The distance to the expansion joint is not mentioned in this document, and is likely to be within 25 cm of the expansion joint, because the impacts of the train wheels also occur within this distance.

In the broadest sense, we dare to define our invention as follows: from the top surface (ie the tread) of the rail head of the rail present in the, preferably for direct resumed operation suited, railroad removing of a piece of rail head so that the rail web and the rail foot, and optionally the lower part of the rail head, remain unaffected, so that in the rail head an at its upper surface debouching hole is created, situated at a distance (preferably of at least 10 mm) from the sides of the rail head (so that the sides of the rail head remain unaffected), and with a prefabricated, shape-retaining, preferably snugly fitting, steel plug filling the hole, wherein, preferably, the shape of the hole and of the plug is congruent, in order, to recover the original geometry of the rail.

By "for direct resumed operation suited railroad" is particularly understood to mean that the to be repaired rail in the operating state remains in the train line, for example, its for safe train traffic necessary mounting to the substrate, and its connection to the in its extension preceding and succeeding rail, for instance by a welded joint such as by welded or joint-free track, is maintained during the repair, so that, for example, the mounting of the damaged rail, is before, during and after the repair work substantially the same. By "upper face of the rail head" is in particular understood to mean the plane that contains the tread for the wheels of the train and at which, respectively, across which the driving wheels of the train rest and drive, so the plane that provides the upper surface thereof during operation of the rail and/or is facing upwards.

The hole is preferably vertical, or up to 10 degrees from the vertical, for example, the hole is made, for example, drilled with a drill, the orientation of which, for example, drill shaft, is vertical, or deviates up to 10 degrees from vertical during the operation, such as drilling.

Preferably, prior to removal of the piece of rail head an inspection is carried out to the rail, to detect a mechanical damage, for example, squat, and the repair is carried out at the site of the damage. In order to detect the damage, for example a measuring or inspection means is used, for example, a scanner (for example, equipped with a light source such as laser), or an image camera or with a magnetic field or electric or acoustic field or other field operating, that is, for example, on board of a vehicle such as a measuring train.

The location of the repair lengthwise of the track will usually be arbitrary and, for example, depend on the result of a damage detection. The distance in rail longitudinal direction will thus be variable with respect to an expansion joint. A repair according to the invention can also be found further than 25 cm from the dilatation joint, for example, more than 50 or 100 or or 150 or 200 cm.

It should be understood that it is preferable to wait for the repair until a damage occurs, which usually occurs only after the track is in use for some time, for example, a minimum of one month or a year or two or five years. The damage is mainly caused by train traffic that drives the railroad.

According to a preferred embodiment of the invention, a piece is removed from the upper part of the rail head of a steel rail situated in the railroad so that a hole is formed in the tread band while the lower portion of the rail head, the rail web and the rail foot are not affected. The hole is then filled with a prefabricated, tightly fitting and form-stable plug of steel which is permanently fixed to the surrounding material of the rail head in order to restore the original geometry of the rail. Preferably, securing involves an interference fit, for instance in that the plug in a shrunken state, for example in that it is significantly colder, for example at least 50 or 100 or 150 degrees Centigrade colder (e.g., cooled by liquid CO2 or N2 or 02), then to be repaired rail, is placed in the hole.

If in the shrunken state, the plug having a diameter equal to or slightly smaller than the hole diameter is placed in the hole and subsequently the plug is allowed to expand, for instance in that the plug heats up to the temperature of the rail head, so that the plug diameter is trying to increase and thus the plug clamps into the hole.

Alternatively, the plug is placed unshrunken, with the plug diameter initially greater than the hole diameter and by insertion into the hole is forced by the hole wall to decrease in diameter.

An effect of which the invention likely makes use is that the wheels of a passing train, locally knead the steel in the upper layer of the top surface of the rail head in the area of contact between the running face of the wheel, and the rail head, so that the inserted plug and the material of the rail head around there experience cold plastic deformation and thus fuse cold. Thus, the plug will fit increasingly better into the hole and all gaps between the hole and the plug smoothly close. Thus it is sufficient to insert a dimensionally stable (or shape-stable) plug into a dimensionally stable (or shape-stable) hole without the use of shape free auxiliary material such as adhesive or molten steel to provide a durable, corrosion resistant fixation of the plug in the hole.

For the plug, one or more of the following applies: cylindrical or parallelepipedic; height greater than 5 or 10 mm and/or less than 30 or 20 or 15 mm; diameter greater than 5, or 10 mm and/or less than 40 or 30 or 25 mm; Contiguous edges are perpendicular to each other; an axial taper of not more than 3, 2 or 1 degrees; of an alloy substantially identical with those of the rail head; one or more of tensile strength, yield point, elongation at rupture and hardness, is substantially equal or greater to that of the rail head; flat bottom and/or top side; contains one or more of Fe, Cr, Mn, Si.

For the hole one or more of the following applies: cylindrical or parallelepiped; depth greater than 5 or 10 mm and/or less than 30 or 20 or 15 mm; depth less than 50% of the height of the rail head; diameter greater than 5 or 10 mm and/or less than 40 or 30 or 25 mm; diameter less than 50% of the width of the rail head; Contiguous edges are perpendicular to each other; an axial taper of no more than 3, 2 or 1 degrees; at least 10 or 15 or 20 mm distance from the sides of the rail head; is located in the contact area between the drive or running surface of the wheels of the train and the upper surface of the rail head; made by spark machining or drilling or milling, or other machining, preferably milling with a milling tool so that a flat hole bottom is created, and after milling the hole bottom and wall are not exposed to a the quality, in particular, the accuracy of one or more of roundness, depth and the diameter of the hole improving mechanical machining with a tool and/or with a milling tool of which the diameter is equal to the hole diameter; made with an indeed or not to center cutting mill; in depth and/or diameter smaller than that of the plug at the same temperature, preferably at least 0.005 mm at 20 degrees Celsius; flat bottom.

The shape of the hole and the plug are preferably adjusted to each other such that when the plug is inserted into the hole, the bottom and/or side walls of the hole and plug make large-scale intimate contact with each other.

Preferably, it is ensured that after the placing of the plug is completed, the upper surface of the plug protrudes slightly above the upper side (the top side is the tread band) of the rail head, preferably at least 0.05 and/or less than 0.1 mm, and then the upper surface of the plug is reduced by a machining operation such as grinding or sanding so that the upper surface of the plug comes to lie flush with the upper surface of the rail head.

In an alternative, it is conceivable that the plug is located in the hole in a sunk state, and after the placing of the plug is completed liquid steel is poured onto the plug in the hole so that the sink above the plug is completely filled with the initially shape free steel.

For example, the plug is driven into the hole by hammering or pressing.

This repair is particularly suitable for so-called. squats. A squat or other damage of the tread band is detected in the rail of the railway taken into operation, is removed by making the hole with a diameter and depth so that the damaged area is completely removed, then the gap is filled up with the plug.

This repair is primarily intended for one or more of: welded or jointless track; rail curve; switch, for example, frog or stock rail or tongue.

This repair is primarily intended for a rail with one of the following steel alloys: manganese steel; Hadfield steel; rail according to EN 13674-1 and/or ProRail RLN 00127-1; Steel with apart from one or more other elements, constituents and/or impurities, Fe (iron) and one or more of: C (carbon); Si (silicon); Mn (manganese); Cr (chromium).

The hardness (Brinell) of the track head and/or the driving surface is preferably at least 200 or 220 or 250 or 260 or 300 or 320 or 350 or 370 or 375 or 400. The rail may be heat treated.

The preferred amounts present in the steel (in wt.%) are as follows: Fe is the main component, for example at least 50% or 80%. C: minimum 0.3 or 0.4 or 0.5 or 0.6 or 0.7 or 0.9 and/or up to 0.6 or 0.8 or 1 or 1.1 or 1.2 or 1, 3 or 1.5. Si: minimum 0.1 or 0.15 or 0.2 or 0.4 or 0.5 and/or up to 0.6 or 0.8 or 1 or 1.1 or 1.2 or 1.5. Mn: minimum 0.1 or 0.5 or 0.7 or 0.8 or 1 or 1.3 and/or up to 1.1 or 1.2 or 1.3 or 1.7 or 2. Cr: minimum 0 , 1 or 0.2 or 0.4 or 0.8 and/or up to 0.15 or 0.3 or 0.6 or 1.2 or 1.5 or 2.

The rail to be repaired is, for example, of Vignole type or grooved rail type, for example, UIC54 or UIC60 or S33 or EB63 or MRS73 or PRI85 and/or has a weight of at least 40 or 45 or 50 kilos per linear meter. For example, the repair is performed to jointless track and/or a track for which the neutral temperature is between 20 and 27, for example is 23, 24, 25 or 26 degrees Celsius.

| **%C** | **%Si** | **%Mn** | **%Cr** |
|---|---|---|---|
| 0,40-0,60 | 0,15-0,58 | 0,70-1,20 | max. 0,15 |
| 0,50-0,60 | 0,20-0,60 | 1,00-1,25 | 0,80-1,20 |
| 0,62-0,80 | 0,15-0,60 | 1,30-1,70 | max. 0,30 |
| 0,55-0.75 | 0,50-1,10 | 0,80-1,20 | 0,40-0,60 |
| 0,60-0,80 | 0,40-1,00 | 0,70-1,10 | max. 0,60 |
| 0,72-0,80 | max. 0,80 | 0,80-1,10 | max. 0,30 |
| 0,70-0,82 | | 1,00-1,30 | |
| 0,72-0,82 | | | |
| 0,90-1,05 | | | |

This table gives examples of preferred ranges for the elements C, Si, Mn and Cr in wt.%, Other combinations and permutations are possible. For example,% C0,62-0,80 combined with% Si0,20-0,60, no Mn and Cr.

Hereinafter, the invention is illustrated by means of an example shown in the drawing. Other embodiments are also included in the invention. Shown in:
Fig. 1 in side elevation view a rail with a defect
Fig. 2 shows the section II-II of Fig. 1
Fig. 3 a side view of the hole in the rail
Fig. 4 in perspective the rail with defect;
Fig. 5 shows the rail of Figure 4 with the hole;
Fig. 6 the track of Fig. 1, repaired.

The rail 10 has a foot 12, web 13 and head 14. The head 14 includes a squat 15 caused by the train wheels. From the tread surface 50 is machined a vertical hole 20 at the place of the squat 15 (FIG. 3).

The defect 15 is located, is removed so that a cylindrical hole 20 is formed, a precisely fitting, slightly upwards protruding plug 21 is placed in the hole, the top of the plug is machined with a tool 120 (Fig. 6), so that a smooth riding surface is obtained.

Fig. 3 shows dotted the wedge-shaped repair described in WO2011119238A1 which extends through the entire rail head and continues into the rail web. This clearly shows the difference with our invention.

Fig. 3 also shows in sectional side view a detail of the rail head to show the pure cylindrical shape of the hole.

## Claims

1. A method of in situ repairing of a defect in a rail (10), wherein in the upper face of the rail head (14) a hole (20) is made by removing rail material, so that the rail web (13) and the rail foot (12), and optionally the lower part of the rail head (14) remain unaffected, so that in the rail head (14) a hole is created that debouches at its upper surface, located at a distance from the sides of the rail head (14) so that the sides of the rail head remain unaffected, and with a preformed shape-stable, preferably closely fitting, steel plug (21) filling of the hole, preferably the shape of the hole (20) and of the plug (21) being congruent in order to restore the original geometry of the rail.

2. A method according to claim 1, wherein the hole (20) is a blind hole and/or the hole is located at a distance of at least 10 mm from the sides of the rail head.

3. A method according to claim 1 or 2, wherein the piece of rail head to be removed contains a damage such as a crack, in particular, a squat.

4. A method according to any one of claims 1-3, wherein the piece of rail head is located at a location that is determined by a preliminary to the repair carried out inspection of the rail head, preferably by a measurement or inspection means moving along the track.

5. A method according to any one of claims 1-4, wherein after the placing of the plug (21) is completed, the top surface of the plug (21) projects slightly above the top of the rail head (14), preferably at least 0.05 and/or less than 0.1 mm, and then preferably the upper surface of the plug (21) is lowered by a machining operation such as grinding or sanding so that the top surface of the plug (21) will be flush with the top surface of the rail head; and/or the hole is made in the tread surface (50) of the train wheels.

6. A method according to any one of claims 1-5, wherein prior to removal of the piece of rail head an inspection is performed on the rail, to detect a mechanical damage thereto, for example, a squat, and the repair is carried out at the site of the damage.

7. A method according to claim 6, wherein to detect the damage a measuring or inspection means is used, in particular, a scanner, preferably equipped with a light source such as laser, or an image camera or with a magnetic field or electric or acoustic field or other field operating, that is, optionally, on board of a vehicle, such as a measuring train.

8. A method according to any one of claims 1-7, wherein in a steel rail situated in the railroad a piece is removed from the upper face of the rail head so that a hole (20) is created in the tread face (50) and the lower portion of the rail head, wherein the rail web (13) and the rail foot (12) remain unaffected, the hole (20) is then filled with a prefabricated, closely fitting and form-retaining steel plug (21) that is permanently attached to the surrounding material of the rail head (14) to restore the original geometry of the rail, wherein, preferably, the attachment is a clamping fit, preferably the plug being applied to the hole in a shrunken state, preferably at a temperature of at least 50 or 100 or 150 degrees Celsius colder than the rail to be repaired, wherein preferably the plug is cooled by liquid CO2, N2 or 02.

9. A method according to any one of claims 1-8, while in the temporary shrunken state the plug, with a diameter being equal to or slightly smaller than the hole diameter, is placed in the hole after which the plug is allowed to expand, for instance in that the plug heats up to the temperature of the rail head so that the plug diameter seeks to increase and thus the plug becomes jammed into the hole.

10. A method according to any one of claims 1-9, wherein for the plug one or more of the following applies: a cylindrical or parallelepiped; height greater than 5 or 10 mm and/or less than 30 or 20 or 15 mm; diameter greater than 5 or 10 mm and/or less than 40 or 30 or 25 mm; contiguous edges are perpendicular to each other; an axial taper of no more than 3, 2 or 1 degrees; of an alloy substantially identical to that of the rail head; one or more of tensile strength, yield strength, elongation at break and hardness substantially equal to or greater than that of the rail head; flat bottom and/or top; contains one or more of Fe, Cr, Mn, Si.

11. A method according to any one of claims 1-10, wherein for the hole one or more of the following applies: a cylindrical or parallelepiped; a depth greater than 5 or 10 mm and/or less than 30 or 20 or 15 mm; depth less than 50% of the height of the rail head; diameter greater than 5 or 10 mm and/or less than 40 or 30 or 25 mm; diameter less than 50% of the width of the rail head; contiguous edges are perpendicular to each other; an axial taper of no more than 3, 2 or 1 degrees; at least 10 or 15 or 20 mm distance from the sides of the rail head; is located in the contact area between the driving or tread face of the wheels of the train and the upper surface of the rail head; made by spark milling or drilling or milling or another machining operation, preferably milling with a milling tool to create a flat hole bottom and after milling the hole bottom and wall are not exposed to a the quality, in particular, the accuracy of one or more of roundness, depth and the diameter of the hole improving mechanical machining with a tool and/or with a milling tool of which the diameter is equal to the hole diameter; made with an indeed or not to center cutting mill; in depth and/or diameter smaller than that of the plug at the same temperature, preferably at least 0.005 mm at 20 degrees Celsius; flat bottom.

12. A method according to any one of claims 1-11, applied to one or more of: welded or jointless track; rail curve; switch, for example, frog or stock rail or tongue.

13. A method according to any one of claims 1-12, the hole being vertical, or up to 10 degrees from the vertical oriented, and/or is made with a tool, the orientation of which during making the recess is oriented vertical, or deviates up to 10 degrees from vertical.

14. A method according to any one of claims 1-13, the repair is carried out:
a) at a distance to the dilatation joint beyond 50 or 100 or 150 or 200 cm: and/or
b) after the track is used for intensive train traffic for a minimum of one month or a year or two or five years.

15. A rail of steel obtained by the repair as claimed in any one of claims 8-14 wherein a damaged rail (10) is provided, wherein the head (14) of the rail comprises a hole (20) which corresponds to a piece removed from the damaged area, wherein the hole (20) is located at a distance from the sides of the rail head, so that the sides of the rail head remain unaffected, wherein the hole (20) that was created in the tread face (50) such that the lower portion of the rail head, the rail web (13) and the rail foot (12) remained unaffected, is filled with a prefabricated, closely fitting and form-retaining steel plug (21) that is permanently attached to the surrounding material of the rail head to restore the original geometry of the rail, wherein the attachment is a clamping fit.

## Patentansprüche

1. Verfahren zur In-situ-Reparatur eines Defektes an einer Schiene (10), wobei in der Oberseite des Schienenkopfes (14) ein Loch (20) gemacht wird, indem Schienenmaterial entfernt wird, so dass der Schienensteg (13) und der Schienenfuß (12) und optional der untere Teil des Schienenkopfes (14) unbeeinflusst bleiben, so dass in dem Schienenkopf (14) ein Loch erzeugt wird, welches an seiner Oberseite hervortritt, und zwar angeordnet in einer Distanz von den Seiten des Schienenkopfes (14) so, dass die Seiten des Schienenkopfes unbeeinflusst bleiben, und wobei ein vorgeformter formstabiler vorzugsweise eng passender Stahlstöpsel (21) das Loch füllt, wobei vorzugsweise die Form des Loches (20) und des Stöpsels (21) kongruent sind, um die ursprüngliche Geometrie der Schiene wieder herzustellen.

2. Verfahren nach Anspruch 1, wobei das Loch (20) ein Sackloch ist und/oder wobei das Loch in einer Distanz von mindestens 10 mm von den Seiten des Schienenkopfes angeordnet ist.

3. Verfahren nach Anspruch 1 oder 2, wobei der Teil des Schienenkopfes, der entfernt werden soll, einen Schaden aufweist, wie beispielsweise einen Riss, insbesondere eine Vertiefung.

4. Verfahren nach einem der Ansprüche 1-3, wobei der Teil des Schienenkopfes an einer Stelle angeordnet ist, die durch eine Vorprüfung vor der Reparatur bestimmt wurde, die durch eine Inspektion des Schienenkopfes ausgeführt wurde, vorzugsweise durch eine Messung oder Inspektionsmittel, die sich entlang der Schiene bewegen.

5. Verfahren nach einem der Ansprüche 1-4, wobei, nachdem das Einsetzen des Stöpsels (21) vollendet ist, die Oberseite des Stöpsels (21) geringfügig über die Oberseite des Schienenkopfes (14) vorsteht, vorzugsweise mindestens 0,05 mm und/oder weniger als 0,1 mm, und wobei dann vorzugsweise die Oberseite des Stöpsels (21) durch eine maschinelle Bearbeitung abgesenkt bzw. abgeflacht wird, wie beispielsweise durch Schleifen oder Abtragen, so dass die Oberseite des Stöpsels (21) bündig mit der Oberseite des Schienenkopfes sein wird; und/oder wobei das Loch in der Lauffläche (50) der Schienenräder gemacht wird.

6. Verfahren nach einem der Ansprüche 1-5, wobei vor der Entfernung des Teils des Schienenkopfes eine Inspektion an der Schiene ausgeführt wird, um einen mechanischen Schaden daran zu detektieren, beispielsweise eine Vertiefung, und wobei die Reparatur am Ort des Schadens ausgeführt wird.

7. Verfahren nach Anspruch 6, wobei zur Detektion des Schadens eine Messung oder ein Inspektionsmittel verwendet wird, insbesondere ein Scanner bzw. Abtastgerät, vorzugsweise ausgerüstet mit einer Lichtquelle, wie beispielsweise einem Laser oder einer Bildkamera, oder mit einem Magnetfeld oder einem elektrischen oder akustischen Feld oder einem anders arbeitenden Feld, welches optional auf einer Platte eines Fahrzeugs ist, wie beispielsweise einem Messzug.

8. Verfahren nach einem der Ansprüche 1-7, wobei bei einer Stahlschiene, die in dem Gleis angeordnet ist, ein Teil von der Oberseite des Schienenkopfes entfernt wird, so dass ein Loch (20) in der Lauffläche (50) und dem unteren Teil des Schienenkopfes erzeugt wird, wobei der Schienensteg (13) und der Schienenfuß (12) unbeeinflusst bleiben, wobei das Loch (20) dann mit einem vorfabrizierten eng passenden und formhaltenden Stahlstöpsel (21) gefüllt wird, der permanent an dem umgebenden Material des Schienenkopfes (14) befestigt wird, um die ursprüngliche Geometrie der Schiene wieder herzustellen, wobei die Befestigung vorzugsweise eine Presspassung ist, wobei der Stöpsels vorzugsweise in das Loch in einem geschrumpften Zustand eingebracht wird, vorzugsweise bei einer Temperatur von mindestens 50 oder 100 oder 150 Grad Celsius kälter als die zu reparierende Schiene, wobei der Stöpsel vorzugsweise durch flüssiges CO₂, N₂ oder O₂ gekühlt wird.

9. Verfahren nach einem der Ansprüche 1-8, wobei in dem temporär geschrumpfte Zustand der Stöpsel mit einem Durchmesser, der gleich oder geringfügig kleiner als der Durchmesser des Loches ist, in dem Loch angeordnet wird, wobei danach gestattet wird, dass der Stöpsel sich ausdehnt, beispielsweise dadurch, dass der Stöpsel sich auf die Temperatur des Schienenkopfes aufheizt, so dass der Durchmesser des Stöpsels versucht zuzunehmen und somit der Stöpsel in das Loch gepresst wird.

10. Verfahren nach einem der Ansprüche 1-9, wobei für den Stöpsel ein oder mehrere der Folgenden zutrifft: zylindrisch oder parallelepipedförmig; Höhe größer als 5 oder 10 mm und/oder geringer als 30 oder 20 oder 15 mm; Durchmesser größer als 5 oder 10 mm und/oder geringer als 40 oder 30 oder 25 mm; anliegende Kanten sind senkrecht zueinander; axiale Verjüngung von nicht mehr als 3, 2 oder 1 Grad; aus einer Legierung, die im Wesentlichen identisch mit jener des Schienenkopfes ist; ein oder mehrere von Zugfestigkeit, Dehnfestigkeit, Bruchlängung und Härte im Wesentlichen gleich oder größer als jene des Schienenkopfes; flacher Boden und/oder Oberteil; enthält eines oder mehrere von Fe, Cr, Mn, Si.

11. Verfahren nach einem der Ansprüche 1-10, wobei für das Loch eines oder mehrere der Folgenden zutrifft: zylindrisch oder parallelepipedförmig; Tiefe größer als 5 oder 10 mm und/oder geringer als 30 oder 20 oder 15 mm; Tiefe geringer als 50% der Höhe des Schienenkopfes; Durchmesser größer als 5 oder 10 mm und/oder geringer als 40 oder 30 oder 25 mm; Durchmesser geringer als 50% der Breite des Schienenkopfes; anliegende Kanten sind senkrecht zueinander; axiale Verjüngung von nicht mehr als 3, 2 oder 1 Grad; mindestens 10 oder 15 oder 20 mm Distanz von den Seiten des Schienenkopfes; in dem Kontaktbereich zwischen der Antriebs- oder Lauffläche der Räder der Schiene und der Oberseite des Schienenkopfes; hergestellt durch Funkenerosion oder Bohren oder Fräsen oder einen anderen maschinellen Bearbeitungsvorgang; vorzugsweise Fräsen mit einem Fräswerkzeug zur Erzeugung eines Lochs mit flachem Boden und wobei nach dem Fräsen der Boden und die Wand des Loches nicht zu einer Qualität freigelegt sind, wobei insbesondere die Genauigkeit von einem oder mehreren der Rundheit, Tiefe und des Durchmessers des Loches, die mechanische Bearbeitung mit einem Werkzeug verbessern und/oder mit einem Fräswerkzeug, dessen Durchmesser gleich dem Lochdurchmesser ist; hergestellt mit einem Indeed bzw. Ausbohrer oder nicht mittigen Schneidfräswerkzeug; bezüglich der Tiefe und/oder des Durchmessers kleiner als jene des Stöpsels bei der gleichen Temperatur, vorzugsweise um mindestens 0,005 mm bei 20 Grad Celsius; flacher Boden.

12. Verfahren nach einem der Ansprüche 1-11, welches bei einem oder mehreren von Folgenden angewendet wird: geschweißtes oder nahtloses Gleis; Schienenkurve; Weiche, beispielsweise Radlenkeraußenschiene oder Zunge.

13. Verfahren nach einem der Ansprüche 1-12, wobei das Loch vertikal oder auf bis zu 10 Grad von der Vertikalen orientiert ist und/oder mit einem Werkzeug gemacht ist, wobei die Orientierung davon während der Herstellung der Vertiefung vertikal orientiert ist oder um bis zu 10 Grad von der Vertikalen abweicht.

14. Verfahren nach einem der Ansprüche 1-13, wobei die Reparatur ausgeführt wird:
a) in einer Distanz zu der Dehnungsverbindung über 50 oder 100 oder 150 oder 200 cm, und/oder
b) nachdem die Schiene für intensiven Bahnverkehr für ein Minimum von einem Monat oder einem Jahr oder zwei oder fünf Jahre verwendet wurde.

15. Schiene aus Stahl, die durch die Reparatur nach einem der Ansprüche 8-14 erhalten wurde, wobei eine beschädigte Schiene (10) vorgesehen ist, wobei der Kopf (14) der Schiene ein Loch (20) aufweist, welches einem Teil entspricht, welches von dem beschädigten Bereich entfernt wurde, wobei das Loch (20) in einer Distanz von den Seiten des Schienenkopfes angeordnet ist, so dass die Seiten des Schienenkopfes unbeeinflusst bleiben, wobei das Loch (20), welches in der Lauffläche (50) erzeugt wurde, so dass der untere Teil des Schienenkopfes, der Schienensteg (13) und der Schienenfuß (12) unbeeinflusst bleiben, mit einem vorfabrizierten eng passenden und formhaltenden Stahlstöpsel (21) gefüllt wird, der dauerhaft an dem umgebenden Material des Schienenkopfes befestigt wird, um die ursprüngliche Geometrie der Schiene wieder herzustellen, wobei die Befestigung eine Presspassung ist.

## Revendications

1. Procédé de réparation in situ d'un défaut dans un rail (10), dans lequel un trou est réalisé dans la face supérieure du champignon de rail (14) par enlèvement de matière du rail, de telle sorte que l'âme de rail (13) et le patin de rail (12), et facultativement la partie inférieure du champignon de rail (14), restent non affectés, de telle sorte que, dans le champignon de rail (14), est créé un trou, lequel débouche à sa surface supérieure, situé à une distance des côtés du champignon de rail (14) de telle sorte que les côtés du champignon de rail restent non affectés, et avec un bouchon en acier (21), de forme stable préformé, de préférence à ajustement étroit, remplissant le trou, de préférence les formes du trou (20) et du bouchon (21) étant congruentes afin de rétablir la géométrie d'origine du rail.

2. Procédé selon la revendication 1, dans lequel le trou (20) est un trou borgne et/ou le trou est situé à une distance d'au moins 10 mm des côtés du champignon de rail.

3. Procédé selon la revendication 1 ou 2, dans lequel le morceau de champignon de rail devant être enlevée contient un dommage tel qu'une fissure, en particulier un squat.

4. Procédé selon l'une quelconque des revendications 1 à 3, dans lequel le morceau de champignon de rail est situé à un emplacement qui est déterminé par une inspection du champignon de rail réalisée avant la réparation, de préférence par un moyen de mesure ou d'inspection se déplaçant le long de la voie.

5. Procédé selon l'une quelconque des revendications 1 à 4, dans lequel, une fois que la mise en place du bouchon (21) est terminée, la surface supérieure du bouchon (21) fait légèrement saillie au-dessus du sommet du champignon de rail (14), de préférence d'au moins 0,05 mm et/ou de moins de 0,1 mm puis, de préférence, la surface supérieure du bouchon (21) est abaissée par une opération d'usinage, telle qu'un meulage ou un sablage, de telle sorte que la surface supérieure du bouchon (21) sera à fleur avec la surface supérieure du champignon de rail ; et/ou le trou est réalisé dans la surface de table de roulement (50) des roues de train.

6. Procédé selon l'une quelconque des revendications 1 à 5, dans lequel, avant enlèvement du morceau de champignon de rail, une inspection est réalisée sur le rail pour détecter un dommage mécanique de celui-ci, par exemple un squat, et la réparation est réalisée à l'emplacement du dommage.

7. Procédé selon la revendication 6, dans lequel, pour détecter le dommage, un moyen de mesure ou d'inspection est utilisé, en particulier un scanneur, de préférence équipé d'une source de lumière telle qu'un laser, ou une caméra d'image ou avec un champ magnétique ou un champ électrique ou acoustique ou un autre champ fonctionnant, qui est, facultativement, à bord d'un véhicule, tel qu'un train de mesure.

8. Procédé selon l'une quelconque des revendications 1 à 7, dans lequel, dans un rail en acier situé dans la voie ferrée, un morceau est enlevé de la face supérieure du champignon de rail de telle sorte qu'un trou (20) est créé dans la face de table de roulement (50) et que la partie inférieure du champignon de rail, l'âme de rail (13) et le patin de rail (12) restent non affectés, le trou (20) étant alors rempli avec un bouchon en acier (21) à conservation de forme et à ajustement étroit, préfabriqué, qui est fixé de manière permanente au matériau environnant du champignon de rail (14) pour rétablir la géométrie d'origine du rail et, de préférence la fixation est un ajustement serré, de préférence le bouchon étant appliqué au trou dans un état rétracté, de préférence à une température d'au moins 50 ou 100 ou 150 degrés Celsius, plus froide que celle du rail devant être réparé, de préférence le bouchon étant refroidi par du O2, N2 ou CO2 liquide.

9. Procédé selon l'une quelconque des revendications 1 à 8, dans lequel, tout en étant dans l'état rétracté temporaire, le bouchon, ayant un diamètre égal ou légèrement inférieur au diamètre de trou, est placé dans le trou, après quoi le bouchon est autorisé à se dilater, par exemple par le fait que le bouchon se réchauffe jusqu'à atteindre la température du champignon de rail de telle sorte que le diamètre de bouchon cherche à s'accroître et, de ce fait, le bouchon se bloque dans le trou.

10. Procédé selon l'une quelconque des revendications 1 à 9, dans lequel, pour le bouchon, un ou plusieurs de ce qui suit s'appliquent : une forme cylindrique ou parallélépipédique ; une hauteur de plus de 5 ou 10 mm et/ou de moins de 30 ou 20 ou 15 mm ; un diamètre de plus 5 ou 10 mm et/ou de moins de 40 ou 30 ou 25 mm ; des bords contigus sont perpendiculaires l'un à l'autre ; une conicité axiale de pas plus de 3, 2 ou 1 degrés ; fait d'un alliage sensiblement identique à celui du champignon de rail ; un ou plusieurs parmi une résistance à la traction, une limite d'élasticité, un allongement à la rupture et une dureté sont sensiblement égales ou supérieures à celui du champignon de rail ; une partie supérieure et/ou inférieure plate ; contient un ou plusieurs parmi Fe, Cr, Mn et Si.

11. Procédé selon l'une quelconque des revendications 1 à 10, dans lequel, pour le trou, un ou plusieurs de ce qui suit s'appliquent : une forme cylindrique ou parallélépipédique ; une profondeur de plus de 5 ou 10 mm et/ou de moins de 30 ou 20 ou 15 mm ; une profondeur de moins de 50 % de la hauteur du champignon de rail ; un diamètre de plus de 5 ou 10 mm et/ou de moins de 40 ou 30 ou 25 mm ; un diamètre de moins de 50 % de la largeur du champignon de rail ; des bords contigus sont perpendiculaires l'un à l'autre ; une conicité axiale de pas plus de 3, 2 ou 1 degrés ; une distance d'au moins 10 ou 15 ou 20 mm par rapport aux côtés du champignon de rail ; est situé dans la zone de contact entre la face d'entraînement ou de table de roulement des roues du train et la surface supérieure du champignon de rail ; est réalisé par fraisage par étincelage ou perçage ou fraisage ou autre opération d'usinage, de préférence fraisage avec un outil de fraisage pour créer un fond de trou plat et, après le fraisage, la paroi et le fond de trou ne sont pas exposés, la qualité, en particulier la précision d'un ou plusieurs éléments parmi la rondeur, la profondeur et le diamètre du trou subissant un usinage mécanique d'amélioration avec un outil et/ou avec un outil de fraisage dont le diamètre est égal au diamètre de trou ; est réalisé avec une fraise de coupe au centre ou non ; une profondeur et/ou un diamètre inférieur à celui du bouchon à la même température, de préférence d'au moins 0,005 mm à 20 degrés Celsius ; un fond plat.

12. Procédé selon l'une quelconque des revendications 1 à 11, appliqué à un ou plusieurs : une voie soudée ou sans raccord ; une courbe de rail ; un commutateur, par exemple, un cœur de croisement ou un rail ou lame contre-aiguille ou d'aiguillage.

13. Procédé selon l'une quelconque des revendications 1 à 12, le trou étant vertical, ou incliné de jusqu'à 10 degrés par rapport à la verticale, et/ou est réalisé avec un outil dont l'orientation pendant la réalisation de l'évidement est orientée verticalement, ou dévie de jusqu'à 10 degrés par rapport à la verticale.

14. Procédé selon l'une quelconque des revendications 1 à 13, dans lequel la réparation est réalisée :
a) à une distance du joint de dilatation supérieure à 50 ou 100 ou 150 ou 200 cm ; et/ou
b) après que la voie est utilisée pour une circulation ferroviaire intensive pendant un minimum d'un mois ou d'une année ou deux ou cinq ans.

15. Rail en acier obtenu par la réparation selon l'une quelconque des revendications 8 à 14, dans lequel un rail endommagé (10) est fourni, le champignon (14) du rail comprenant un trou (20) qui correspond à un morceau enlevé de la zone endommagée, le trou (20) étant situé à une distance des côtés du champignon de rail, de telle sorte que les côtés du champignon de rail restent non affectés, le trou (20) qui a été créé dans la face de table de roulement (50), de telle sorte que la partie inférieure du champignon de rail, l'âme de rail (13) et le patin de rail (12) restent non affectés, étant rempli avec un bouchon en acier (21) à conservation de forme et à ajustement étroit, préfabriqué, qui est fixé de manière permanente au matériau environnant du champignon de rail pour rétablir la géométrie d'origine du rail, la fixation étant un ajustement serré.
